



oxo-decyl alcohol. The oxo-decyl alcohol as used herein is a decyl alcohol prepared by a conventional oxo-synthesis process. The alcohol is, essentially, a mixture of C<sub>10</sub> isomers. The di-alkyl dithiophosphate was placed in a flask, mixed with boric acid, and heated to a temperature between 210° and 250° F. for one hour. The atmosphere within the flask was purged with nitrogen during the one hour reaction period. Results of an analysis of the boron di-alkyl monothiophosphate are as follows:

|            |       |
|------------|-------|
| Percent B: |       |
| Calc.      | 1.42  |
| Found      | .96   |
| Percent P: |       |
| Calc.      | 12.0  |
| Found      | 11.45 |
| Percent S: |       |
| Calc.      | 12.4  |
| Found      | 15.96 |

The new boron monothiophosphates are, for the most part, oily liquids somewhat soluble in many organic solvents. They are particularly soluble in hydrocarbons. The boron monothiophosphates, when combined with a carrier, such as a spray or such as a dust composition, exert a definite toxicity against arachnids such as, for example, *Tetranychus bimaculatus* (two-spotted spider mite), *Paratetranychus pilosus* (European red mite), *Bryobia praetiosa* (clover mite) as well as certain small homopterous insects such as, for example, aphids. This pesticide gives excellent control of such organisms for extended periods of time.

The new toxicant may be used as a spray or as a dust compound. It may be employed in combination with an inert material carrier such as a finely divided solid, or a solvent liquid. The toxicant may be present in the inert carrier material in relatively high concentrations to provide a concentrate adapted for further dilution. It may also be present in the inert carrier material in dilute form to provide compositions suitable for application without further modification.

The following example illustrates the activity of the boron monothiophosphate as a pesticide:

#### EXAMPLE A

A standard agricultural screening method was used to test the arachnids. The test included both the nymph and adult stage. A contact spray method was used within a Peet-Grady chamber. The chamber was operated at 5 p.s.i.g. One hundred organisms were placed on the bean plants. A concentration of 0.025% toxicant in acetone was sprayed on the bean plant. A count was made after 24 hours.

A standard agricultural screening method was used to test the aphididae family. The test included both the nymph and adult stage. A contact spray method was used within a Peet-Grady chamber. The chamber was operated at 5 p.s.i.g. One hundred organisms were placed on cotton plants. A concentration of 0.1% toxicant in acetone was sprayed on the cotton plant. A count was made after 24 hours.

Results obtained from the pesticide tests follow:

#### Pesticide Tests

| Toxicant                                                               | Aphids,<br>percent<br>kill | Two<br>spotted<br>mite,<br>percent<br>kill |
|------------------------------------------------------------------------|----------------------------|--------------------------------------------|
| Boron di-n-decyl monothiophosphate<br>(obtained from Example I method) | 100                        | 87                                         |
| Boron di-alkyl monothiophosphate<br>(obtained from Example II method)  | 96                         |                                            |

It has been proposed to add minor amounts of boron in the form of soluble or dispersable boron compounds to the liquid hydrocarbon fuels used in internal combustion engines.

Among the compounds previously proposed for such purposes are the tri-alkyl borates and the tri-alkyl borines, such as tri-amyl borine and tri-isobutyl borate. This invention contemplates the addition of a boron compound which is soluble in a liquid hydrocarbon fuel and which compound contains phosphorus as well as boron.

A standard CFR L-head engine test utilizes an engine with a compression ratio of 7.0 to 1, a water temperature of 148° F. (±3° F.), an oil temperature of 160° F. (±3° F.), and an air intake temperature of 110° F. (±5° F.). The test cycle is as follows:

| Cycle            |           |         |
|------------------|-----------|---------|
|                  | Full load | No load |
| Time in seconds. | 135       | 45      |
| Speed, r.p.m.    | 900       | 600     |
| Air/fuel ratio   | 13.0/1    | 11.5/1  |

Data obtained in a standard CFR L-head engine test are as follows:

#### Standard CFR L-Head Engine Test

|                               | Base fuel | Base fuel,<br>2% boron<br>monothio-<br>phosphate | Percent<br>reduction |
|-------------------------------|-----------|--------------------------------------------------|----------------------|
| Surface ignition, counts/min. | 350       | 70                                               | 80                   |

These data demonstrate the utility of the boron monothiophosphate as a liquid hydrocarbon fuel additive.

A di-alkyl monothiophosphate was prepared by the reaction of P<sub>2</sub>S<sub>5</sub> with a mixture of 70 mole percent isopropyl alcohol and 30 mole percent oxo-decyl alcohol and subsequent reaction with boric acid as set forth in Example II. This material was tested in a standard Timken testing machine. Such test is well known to those skilled in the art as being useful in obtaining valuable information with respect to the potential commercial value of extreme pressure lubricants. The Timken machine and test are fully described in the Journal of the Institute of Petroleum, 32, pages 209-210 and 220-222 (1946).

The data obtained for a base oil consisting of SAE-30 petroleum lubricating oil containing 3 weight percent of a barium-containing neutralized phosphorus-sulfide hydrocarbon reaction product detergent from the Timken testing machine are as follows:

#### Timken Test Results

| MATERIAL                 | Load, lbs. |      |
|--------------------------|------------|------|
|                          | Pass       | Fail |
| Base oil                 | 6          | 9    |
| Base oil + 0.5% additive | 35         | 40   |
| Base oil + 0.1% additive | 27         | 30   |

These data demonstrate a substantial improvement in Timken load value resulting from the addition of a very small amount of boron monothiophosphate to a conventional petroleum lubricating oil.

The effectiveness of the boron compounds of the present invention in inhibiting corrosion toward copper, silver and/or lead-containing metals and their oxidation inhibiting properties are demonstrated by data obtained by subjecting samples of the above metals to a Sand Stirring Corrosion Test. In this test a metal test specimen was slightly abraded with steel wool, washed with naphtha, dried and weighed to the nearest mg. The cleaned test coupon was suspended in a steel beaker, cleaned with hot trisodium phosphate solution, rinsed with water, rinsed with acetone, and dried. An oil solution (250 g.) con-

taining 1% di-n-decyl monothiophosphate was placed together with 0.625 g. lead oxide and 50 g. of a 30-35 mesh sand in the beaker. The beaker was then heated to a temperature of 300° F. ( $\pm 2$ ° F.) while the contents of the beaker were stirred by means of a stirrer which rotated at 750 r.p.m. The contents of the beaker were maintained at this temperature and under this condition for 48 hours after which the metal coupon was removed, rinsed with naphtha, dried, and weighed. Results of the test are as follows:

### *Sand Stirring Corrosion Test*

| Material               | Wt. loss, mg. |         |
|------------------------|---------------|---------|
|                        | 48 hrs.       | 72 hrs. |
| Base oil               | 700           | 1,000   |
| Base oil + 1% additive | 55.1          | 71.2    |

While the invention has been described with particular reference to specific embodiments, it is to be understood that the invention is not limited thereto but is to be construed broadly and restricted solely by the scope of the appended claim.

We claim:

A lubricating oil composition consisting essentially of a petroleum lubricating oil and from about 0.1% to about

10% by weight of a boron phosphorus-containing compound having the formula:



10 wherein  $R_1$  and  $R_2$  are each the hydrocarbyl residue of an alcohol of a mixture of alcohols consisting of about 70 mole percent isopropyl alcohol and about 30 mole percent decyl alcohol.

**References Cited in the file of this patent**

UNITED STATES PATENTS

|           |                   |               |
|-----------|-------------------|---------------|
| 2,224,695 | Prutton           | Dec. 10, 1940 |
| 2,346,156 | Farrington et al. | Apr. 11, 1944 |
| 2,721,180 | Lawrence et al.   | Oct. 18, 1955 |
| 2,743,235 | McDermott         | Apr. 24, 1956 |
| 2,786,009 | Pianfetti et al.  | Mar. 19, 1957 |
| 2,809,163 | Cyphers et al.    | Oct. 8, 1957  |
| 2,843,465 | Yust et al.       | July 15, 1958 |
| 2,885,430 | Scherer et al.    | May 5, 1959   |
| 2,890,947 | Annable et al.    | June 16, 1959 |
| 2,920,993 | Fairchild         | Jan. 12, 1960 |
| 2,922,812 | Gilbert et al.    | Jan. 26, 1960 |
| 3,047,607 | Thayer            | July 31, 1962 |